

Sept. 4, 1934.

L. G. NICOLL

1,972,311

METHOD FOR PRODUCING PHOTOGRAPHIC REPRODUCTIONS IN COLOR

Filed July 25, 1931

2 Sheets-Sheet 1

FIG. 1.



FIG. 2.



FIG. 3.



FIG. 4.



Inventor.  
Leonard G. Nicoll  
by *Keard Smith & Tennant.*  
Atty's.

Sept. 4, 1934.

L. G. NICOLL

1,972,311

# METHOD FOR PRODUCING PHOTOGRAPHIC REPRODUCTIONS IN COLOR

Filed July 25, 1931 2 Sheets-Sheet 2



FIG. 6.



FIG. 7.



22

FIG. 8.



Inventor  
Leonard G. Nicoll

by Heard Smith & Tennant.

AttyS.

## UNITED STATES PATENT OFFICE

1,972,311

## METHOD FOR PRODUCING PHOTOGRAPHIC REPRODUCTIONS IN COLOR

Leonard G. Nicoll, Boston, Mass.

Application July 25, 1931, Serial No. 553,081

13 Claims. (Cl. 95-2)

This invention relates to improvements in methods and apparatus for making photographic reproductions in natural colors.

In the art of photography every step forward has been toward the goal of perfect realism. In this progress the development of a practical method of producing prints in natural color has met with a great deal of difficulty. This fact is borne out by appreciating the fact that a great deal more activity has taken place in the development of reproductions in monochrome. No matter how perfectly the tones of a subject are rendered without color the results are at best only approximately accurate reproductions. The importance and desirability of reproducing in color has always been recognized since the realization of true and accurate reproduction could never be attained in any medium but that of color. The failure of existing methods to faithfully reproduce in color, and the failure to produce a method commercially workable has undoubtedly prevented its more universal adoption.

The object of the present invention is to provide a method and apparatus for producing a multiplicity of colored photographic reproductions in which the method may be carried out by one who is not highly skilled, and in which the material employed is always in such physical condition as to be readily handled or treated chemically without fear of injury.

A further object of the invention is to provide a method of producing multi-color photographic reproductions in which every color of which the subject is composed and the black and white which appear in the subject are faithfully reproduced.

A further object of the invention is to provide a process in which the final color reproduction contains two or more elements bearing the fundamental colors of the subject, each of which may be worked readily upon and modified to produce a desired result in the finished reproduction.

In the drawings:

Fig. 1 is a cross sectional view of a transparency in natural color.

Fig. 2 is a cross sectional view of an apparatus for selectively projecting three beams of color representing the fundamental colors of nature upon a printing frame.

Fig. 3 is a cross sectional view through three photographically sensitized elements bearing a panchromatic emulsion.

Fig. 4 is a cross section through three sheets of silver bromide sensitized printing paper of special construction.

Fig. 5 is a cross section of one of the bromide sheets with its emulsion adhering to a temporary support.

Fig. 6 is a cross section through a steaming apparatus used in the process. 60

Fig. 7 is a cross section on line 7-7 Fig. 6.

Fig. 8 is a cross section similar to that shown in Fig. 5 with the paper backing of the bromide sheet removed.

Fig. 9 is a cross section of the finished picture 65 mounted upon a support.

The present invention presents a thoroughly practical method of making accurate full color reproductions photographically. The process makes possible the production of a multiplicity of 70 identical reproductions, and may be carried out upon a commercial quantity production basis.

In order to emphasize the importance and far reaching possibilities of such a process, it is well to discuss the relative characteristics of the multi-color processes as compared to monochromatic representations which are now so commonly in use.

Monochromatic photography has been so prevalent that the absence of color has not been missed 80 by the general public, but once colored photography has been established on a practical commercial basis, monochrome prints will lose much of their present day popularity.

The process comprising the present invention 85 may be adapted readily to making multi-color reproductions by employing two or more fundamental colors. A very satisfactory two color reproduction may be produced. The better quality resulting from the use of three or four fundamental colors warrants the additional labor and 90 materials necessary for such a reproduction. The particular embodiment of the invention herein described will involve the use of three fundamental colors, such, for instance, as the red, the 95 blue and the yellow.

The first step in the process may be carried out by a number of different methods. It has been found, however, that a very satisfactory initial step in the process is to produce a transparency 100 in natural colors of the subject, such for instance, as the well known plate known as the "Autochrome" or the "Agfa" color plate. Since the method of obtaining such a transparency is well known to those skilled in the art, the method will 105 not be described. A photographic record of the fundamental colors in the subject, however, may be obtained by means of various other processes, such as obtaining the appropriate number of negative records by exposure through trichrome fil- 110

ters directly from the subject in which case three separate exposures must be made through a lens or an especially constructed camera must be used which projects images containing the three standard colors upon three separate plates or other panchromatic material.

By the preferred method, however, the color transparency above referred to is used as a basis from which to produce the final reproduction.

10 Three negative records are made upon appropriate panchromatically sensitized material. Each negative record thus made bears an image representing the amount and position of one of the fundamental colors which appear in the subject.

15 A convenient means for obtaining these records is by the use of the apparatus disclosed in Fig. 2. The apparatus is mounted preferably upon a bench or table 1 in which an opening 2 is formed substantially of the same shape and area as the 20 color plate used in the process. A printing frame 3 is placed over the opening 2 in which are received the materials employed in this step of the process. Below the opening 2 is secured a light tight casing 4 upon the lower end of which is 25 secured a frame 5 having a slot 6 therein in which is slidably received a color filter carrying frame 7 which is movable within the slot 5 in a direction parallel to the printing frame 3. Below the frame 5 is secured another frame 8 in which is received 30 an additional color filter. Below the frame 8 is located a light tight chamber 9 containing a light source 10.

To produce the desired negative records, a compensating filter 11 is placed desirably in the 35 frame 8 which acts to cut off a particular part of the spectrum emanating from the light source which is undesirably strong. A set of colored filters then are placed in slots 12, 13 and 14 within the frame 7. These filters preferably are 40 standard trichromatic. The blue filter 15 is placed in the slot 12, the red filter 16 is placed in the slot 13, and the green filter 17 is placed in the slot 14. The particular arrangement of the filters is immaterial however. As shown in 45 the drawing the filter 15 is in position to intercept the light passing from the light source to the printing frame in which is placed the transparency 18 from which the reproduction is to be made. This beam of blue light passes through 50 the transparency and strikes a panchromatically sensitized sheet 19 placed in contact with the transparency, and produces when developed a negative record thereon of that color contained in the transparency complementary to the blue 55 of the filter 15, such complementary color being the yellow. A negative record is made in the same way of the blue and the red contained in the transparency upon separate sensitized sheets by moving the filters 16 and 17 respectively in the position occupied by the filter 15 in the drawings. The records made of the blue and the red are designated respectively 20 and 21.

There are many advantages resulting from the use of a transparency for producing the three 65 negative records 19, 20 and 21 in preference to producing such records by making separate exposures from the subject itself. It is a difficult matter to make three correct exposures directly from the subject especially if there is a possibility of movement in the subject in which case 70 proper registration of the colored sensation prints produced from the negatives is impossible, and in many cases the final result is most unsatisfactory.

75 On the other hand, by the use of a trans-

parency this and many other difficulties are overcome. When using transparencies, there is always the possibility of correcting an over or under exposed negative of any color by making another exposure from the original transparency or the transparency itself may be intensified or reduced either entirely or locally as may be required.

There have been numerous methods devised for making prints in the three primary or fundamental colors. Some of these methods employ the use of dyes, while some of them use pigment prints as in the carbon process, while still other methods employ a combination of both of these processes.

Those conversant with dye processes are aware of the trouble resulting from that use which causes spreading of one color into other colors, and the difficulty of registration of such prints.

The carbon process which produces very beautiful results in the production of monochromatic prints is exceedingly difficult when making three delicate and infinitely fragile prints such as are required for trichrome printing. Registration of

90 such prints when they are superposed presents an enormous difficulty owing to the chance of damage to the prints by reason of their extreme delicacy. The same remarks apply to the "Carbro" process which is an adaptation of the carbon process.

Attempts have been made to use tone prints, but the difficulty so far has been with the red which is never of the required shade, always leaning strongly to a brick red whereas as magenta red is the required tone. Bearing in mind all the foregoing troubles and difficulties, and yet realizing the possibilities of color prints, the present invention provides a method which overcomes these difficulties and makes the production of full color prints a comparatively easy matter.

105 The next step in the process is to print from the three negatives 19, 20 and 21 three positive sensation prints, each bearing a positive record of the amount and position of the standard trichromatic colors contained in the subject.

110 These positive records are made upon especially prepared photographic material illustrated in Fig. 4. This material comprises a hard gelatine layer 22 in which is incorporated a photographically sensitive silver composition, preferably silver bromide. This hard gelatine film is secured to a backing material 23 by means of a layer 24 of relatively soft gelatine. The support 23 may be of any suitable character but is preferably 115 a sheet of backing paper.

120 In Fig. 4 three sensation prints are designated generally as A, B and C. These prints are prepared by exposing for the proper period of time in contact with the negatives 19, 20 and 21 and are thereafter developed in the usual manner.

125 The next step in the process is to secure the sensation prints A, B and C face downward into contact with temporary supports 25. Any suitable material may be used for these supports. A 130 highly desirable material for this purpose is transparent celluloid. The paper prints are soaked in water and squeegeed in the contact with the celluloid sheets which have been previously waxed and are substantially larger in 135 area than the prints themselves which provides a convenient margin, by means of which the prints may be more readily handled.

140 A very important feature of the present invention is the step in the process which permits the 145

gelatine film bearing the positive images to be stripped from their original paper backing, which operation is done as follows. The three prints mounted upon their temporary supports are subjected to a steam bath which softens the readily soluble soft gelatine layer thereby permitting the paper backing sheets 23 to be stripped from the hard gelatine films 22 without injury thereto or modification of the images contained therein.

10 A convenient apparatus in which to carry on this operation is shown in Figs. 6 and 7. The apparatus comprises a casing 29 secured to a bench or table and within which is received a tank 30 containing water, and beneath which is located a gas burner 31 or other suitable heating apparatus which is used to generate steam from the water contained in the tank. The steam passes upwardly through conduits 32 and 33 at the ends of the tank. From this point the steam 20 rises into a steam chamber 34. Above the tank 30 is situated a tray 35 fixed in position and extending across the casing from one end wall to the other. Access to the tray is gained by means of hinged doors 36 and 37 adjacent the 25 ends of the tray 35 and are hinged upon the casing 29 at 38.

The steam passing through the conduits 32 and 33 is directed upward by the baffle plates 39 and 40 from where it passes along the sides of the 30 tray 35 and upwardly into the chamber 34 in which is situated deflecting surfaces 41 which act to direct the steam downwardly into contact with the tray.

To steam the prints one of the doors 36 is 35 opened and a print is placed in the tray 35 and is passed out of the steam bath at the other end of the tray through the opposite door 37. The prints are subjected to the steam for the required length of time to soften the soft gelatine layer 40 to the proper consistency which will permit the paper backing to be stripped from the hard gelatine layer. The stripping operation desirably is accomplished immediately upon withdrawing the prints from the steam bath. The prints are 45 placed in the steaming apparatus with their backing material upwardly and are subjected to the currents of steam directed downwardly by the surfaces 41.

The hard gelatine films are now left adhering 50 to their celluloid supports 25 and the silver images contained therein are ready to be converted into their respective colors. This coloring operation may be carried on before the paper backing 23 is stripped from the gelatine film. If this is 55 done the images are colored after exposure and development, and before waxing into contact with the temporary supports. It is preferable however to color the prints after they have been transferred to their temporary supports as at 60 this time they are more readily handled, and the washing operation consumes much less time.

As has been previously pointed out other methods may be used to color the prints, but the following method has been found to produce the 65 most accurate and permanent reproductions.

Bleach the print which is to be converted into yellow in—

70 Potassium ferricyanide 60 grains  
Lead nitrate 40 grains  
Water 2 ounces

Wash until all stain has disappeared, then tone in—

75 Potassium bichromate 15 grains  
Water 3 ounces

The print which is to be toned blue is placed in the following—

|                         |            |
|-------------------------|------------|
| Ammonium ferric citrate | 22 grains  |
| Nitric acid             | 24 minimis |
| Potassium ferricyanide  | 45 grains  |
| Water                   | 10 ounces  |

The blue image must be well washed to remove the green stain, and, if fixed in plain hypo 5% solution afterwards, a very clear transparent blue print results.

As previously stated, it is not possible to obtain a red print by toning methods, which will be in any way satisfactory but it is quite easy to convert the grey bromide into a magenta print as follows.

The celluloid, holding the print, is soaked in water and a sheet of magenta carbon tissue, cut slightly larger than the bromide print, is sensitized in the "Carbro" or similar, standard baths for the required time. This is then brought into contact with the wet bromide print, squeegeed into perfect contact and pressed for about fifteen minutes.

Instead of separating the bromide and carbon tissue, the celluloid, bearing both is plunged into warm water, when the paper backing of the carbon will separate and can be removed, the remaining gelatine washed away, except for the amount held by the silver image.

After complete development in warm water the celluloid is fixed in an acid hypobath.

|                          |            |
|--------------------------|------------|
| Sodium thiosulphate      | 4 ounces   |
| Potassium metabisulphite | 1/2 ounces |
| Water                    | 20 ounces  |

which removes the bleached bromide image, which would otherwise darken in daylight, and also removes any bichromate stain. After dying the three component prints are ready for assembling. Before doing so, these may be superimposed to see if the color balance is correct. When satisfied that this is so, the three color images can be assembled to make one print.

To do this a piece of double transfer paper 42, slightly larger than the color images, is soaked in water until completely stretched.

This is then squeegeed into contact with the yellow print on celluloid and allowed to dry, or it can be subjected to a draught from an electric fan. When completely dry, the paper, with the color image, will either fall off, or can be peeled off completely from the celluloid.

The wax, with which the celluloid was polished, is now adhering to the surface of the yellow print, and this must be removed by absorbent cotton dipped in benzole.

The yellow print is now placed in cold water again for a few minutes and then squeegeed into contact with the red image and quickly brought into exact register. This is again dried, and removed from the celluloid support, bearing both the yellow and red prints firmly cemented together by cohesion. After cleaning as before, and re-wetting, the two color print is brought into contact with the blue image when all the colors of the original will be found correct.

After drying, removing from the celluloid and cleaning, this print has now a high gloss, which is excellent for reproduction, but, if desired, this can be removed by soaking the finished print in cold water until quite limp, and allowing it to dry in the ordinary way, when the surface will be matt with a pleasant sheen. There are alternative methods, which are equally effective,

and may be preferred for some things. For instance, the bromide print, which is converted into yellow need not be transferred to celluloid, but may be used itself as the foundation print, superposing the other two colors on it.

This will give a final result of a high gloss, and, if matting is desired this must be done afterwards, but it is not necessary in this case to clean the tricolor print, as the wax on its surface ensures the matted print leaving the surface of the ground opal glass (which is best for this purpose) easily.

Another variation is to make all three grey images or their celluloids into color images, by using carbon tricolor tissues for each in the same way as for the red previously.

In this way, however, the yellow print cannot be used for the final support, unless it is well hardened and thoroughly washed before conversion into its yellow state.

A still further variation is to convert the grey bromide prints on the celluloids into dye images but as before mentioned this is not recommended.

25. In all methods of color printing, in which celluloid sheets are used for the temporary supports, it is of undoubted advantage to use a substratum to secure perfect holding of the delicate detail of the color images, but, with the method 30 just described, no substratum is needed, as the film of hardened gelatine acts in the desired way itself.

The three superposed colored films may themselves be used as a transparency, to be viewed 35 by transmitted light or they may be mounted upon a piece of glass or other transparent material 42 to provide mechanical support for the films.

It is more desirable, however, that the films be 40 mounted upon a support having a substantially totally reflecting surface. Such reflecting surface may be pure white or may contain a light tint of a particular color which it is desired to introduce into the reproduction to obtain a desired special effect. For instance, while it is 45 possible to reproduce a subject correctly by the above method, it may be desirable in some cases such as in a snow scene to overemphasize the blue or in views of another character such as a 50 landscape in summer, a green tint may be thus introduced. This may be done by mounting the films upon a support having the blue or the green tint.

Another possibility of controlling the impression created by the reproduction is to use upon 55 the reflecting surface a color compensatory of the variation from daylight of that of the color source which is projected upon the reproduction.

Having thus described the invention, what is 60 claimed as new, and desired to be secured by Letters Patent, is:

1. The method of making photographic reproductions in colors consisting in making two or more photographic records, each bearing a negative image representing the amount and position of a fundamental color as contained in the subject, making two or more sensation positive prints from the negatives upon a gelatine emulsion having a hard layer carrying a photographically sensitive silver composition and a relatively soft layer adherent to a support, each print bearing a positive silver image of its respective color, causing each of the gelatine films to adhere to a transparent temporary support, softening the layer of gelatine adhering to each original support, stripping the original support from each of the gelatine films in the presence of steam, converting each positive image to that color it is to create in the finished reproduction, superposing the films and securing in registered position by cohesion, each temporary backing being removed from its respective film after each superposition.

80. 2. A method of making photographic reproductions in colors consisting in making two or more photographic records, each record bearing a negative image representing the amount and position of a fundamental color as contained in the subject making two or more sensation positive prints from the negatives upon a gelatine emulsion having a hard layer carrying a photographically sensitive silver composition and a relatively soft layer adherent to a support, each print bearing a silver image of its respective color, causing each of the gelatine films to adhere to a transparent temporary support, softening the layer of gelatine adhering to the original support of each of the gelatine films in the presence of steam, converting each positive image to that color it is to create in the finished reproduction superposing each film in the registered position with its soft gelatine layer in a softened tacky condition thereby securing the films in such position by cohesion, each temporary backing being removed after each superposition.

85. 3. The method of making photographic reproductions in colors consisting in making two or more photographic records, each record bearing a negative image representing the amount and 90 position of a fundamental color as contained in the subject making two or more sensation positive prints from the negatives upon a gelatine emulsion having a hard layer carrying a photographically sensitive silver composition and a relatively soft layer adherent to a paper support, each print bearing a positive silver image of its respective color, causing each of the gelatine films to adhere to a transparent temporary support, softening the layer of gelatine adhering to each paper support by subjecting it to the action of steam, stripping the original supports from each of the gelatine films, converting each positive image to that color it is to create in the finished reproduction superposing the films and 95 securing in registered position by cohesion, each temporary backing being removed from its respective film after each superposition.

100. 4. The method of making photographic reproductions in colors consisting in making two or more photographic records upon panchromatically sensitized photographic material by means of appropriate colored filters, each record bearing a negative image representing the amount and position of a fundamental color as contained in the subject making two or more sensation positive prints from the negatives upon a gelatine emulsion having a hard layer carrying a 105 photographically sensitive silver composition and a relatively soft layer adherent to a paper support, each print bearing a positive silver image of its respective color, causing each of the gelatine films to adhere to a transparent temporary support, softening the layer of gelatine adhering to each paper support by subjecting it to the action of steam, stripping the paper supports from each of the gelatine films converting each 110 positive image to that color it is to create in the finished reproduction superposing the films and securing in registered position by cohesion, each temporary backing being removed from its respective film after each superposition and mounting the superposed films upon a support having a substantially totally reflecting surface.

115. 5. The method of making photographic reproductions in colors consisting in making two or more photographic records upon panchromatically sensitized photographic material by means of appropriate colored filters, each record bearing a negative image representing the amount and position of a fundamental color as contained in the subject making two or more sensation positive prints from the negatives upon a gelatine emulsion having a hard layer carrying a 120 photographically sensitive silver composition and a relatively soft layer adherent to a paper support, each print bearing a positive silver image of its respective color, causing each of the gelatine films to adhere to a transparent temporary support, softening the layer of gelatine adhering to each paper support by subjecting it to the action of steam, stripping the paper supports from each of the gelatine films converting each 125 positive image to that color it is to create in the finished reproduction superposing the films and securing in registered position by cohesion, each temporary backing being removed from its respective film after each superposition and mounting the superposed films upon a support having a substantially totally reflecting surface.

130. 6. The method of making photographic reproductions in colors consisting in making two or more photographic records upon panchromatically sensitized photographic material by means of appropriate colored filters, each record bearing a negative image representing the amount and position of a fundamental color as contained in the subject making two or more sensation positive prints from the negatives upon a gelatine emulsion having a hard layer carrying a 135 photographically sensitive silver composition and a relatively soft layer adherent to a paper support, each print bearing a positive silver image of its respective color, causing each of the gelatine films to adhere to a transparent temporary support, softening the layer of gelatine adhering to each paper support by subjecting it to the action of steam, stripping the paper supports from each of the gelatine films converting each 140 positive image to that color it is to create in the finished reproduction superposing the films and securing in registered position by cohesion, each temporary backing being removed from its respective film after each superposition and mounting the superposed films upon a support having a substantially totally reflecting surface.

145. 7. The method of making photographic reproductions in colors consisting in making two or more photographic records upon panchromatically sensitized photographic material by means of appropriate colored filters, each record bearing a negative image representing the amount and position of a fundamental color as contained in the subject making two or more sensation positive prints from the negatives upon a gelatine emulsion having a hard layer carrying a 150 photographically sensitive silver composition and a relatively soft layer adherent to a paper support, each print bearing a positive silver image of its respective color, causing each of the gelatine films to adhere to a transparent temporary support, softening the layer of gelatine adhering to each paper support by subjecting it to the action of steam, stripping the paper supports from each of the gelatine films converting each positive image to that color it is to create in the finished reproduction superposing the films and securing in registered position by cohesion, each temporary backing being removed from its respective film after each superposition and mounting the superposed films upon a support having a substantially totally reflecting surface.

- to create in the finished reproduction, superposing the films and securing in registered position by cohesion each temporary backing being removed from its respective film after each superposition. 5. The method of producing a photographic reproduction in natural colors consisting in making a transparency in natural colors by a photographic process contact printing three or more negative records from the transparency by inserting in the path of a light source suitable colored filters, each negative record representing the amount and position of one of the fundamental colors contained in the transparency 10 15 20 25 30 35 40 45 50 55 60 65 70 75 80 85 90 95 100 105 110 115 120 125 130 135 140 145
- record bearing a negative image representing the amount and position of a fundamental color as contained in the subject, making two or more sensation positive prints from the negatives upon a gelatine emulsion having a hard layer carrying a photographically sensitive silver composition and a relatively soft layer adherent to a support, each print bearing a positive silver image of its respective color, converting each positive image to that fundamental color it is to create in the finished reproduction, causing each of the gelatine films to adhere to a transparent temporary support softening the layer of gelatine adhering to each of the original supports by subjecting it to the action of steam, stripping the original supports from each of the gelatine films, superposing the films and securing in registered position by cohesion, each temporary backing being removed from its respective film after each superposition. 9. The method of making photographic reproductions in natural colors comprising the steps defined in claim 8 together with mounting the superposed gelatine films upon a transparent support permitting the reproduction to be viewed by transmitted light. 10. The method of making photographic reproductions in natural colors comprising the steps defined in claim 8 together with mounting the superposed gelatine films upon a support having a surface which is substantially totally reflecting. 11. Steps in the process of producing photographic reproductions in natural colors which consists in producing a film which comprises a gelatine emulsion having a hard layer carrying a photographically sensitized silver composition and a relatively soft gelatine layer adherent to a support making a photographic record upon said sensitized layer releasing said hard layer from said support by the action of steam upon said soft gelatine layer. 12. Steps in the process of producing photographic reproductions in color which consists in printing a positive image representing the amount and position of a fundamental color of the subject upon a gelatine emulsion having a hard layer carrying a photographically sensitive composition and a relatively soft layer adherent to a support, releasing said hard layer from said support by the action of steam upon said soft gelatine layer. 13. Steps in the process of making photographic reproductions in colors which consist in printing a positive image representing the amount and position of a different primary color of the subject upon each of a plurality of gelatine emulsions, each emulsion having a hard layer carrying a photographically sensitive composition and a relatively soft layer adherent to a paper backing, releasing said hard layer from said paper backing by the action of steam upon said soft gelatine layer and superposing said layers of hard gelatine emulsions with their images in registry while the soft gelatine layer remaining upon the hard layer is still in a tacky condition. 8. The method of producing photographic reproductions in natural colors consisting in making three or more photographic records, each

LEONARD G. NICOLL.